

1

3,247,148  
ELECTROSTATIC COMPOSITIONS COMPRISING  
SODIUM SALT OF MAHOGANY SULFONIC  
ACID, POLAR SOLVENTS AND WATER  
William H. Ellis, El Segundo, and Valeria Artel, Los  
Angeles, Calif., assignors to Chevron Research Com-  
pany, a corporation of Delaware  
No Drawing. Filed Sept. 23, 1963, Ser. No. 310,904  
6 Claims. (Cl. 260—29.2)

This invention concerns novel electrostatic conductivity additives and compositions containing them. Specifically, it pertains to additives consisting of oil-soluble sulfonates, water and polar solvents which are used in electrostatic coating compositions.

A substantial portion of industrial paints are now applied electrostatically. This method of application consists of utilizing a high-voltage, low-current mechanism to atomize and charge the coating compositions. The spray particles of the coating compositions carry a negative charge, whereas the object to be coated is positively charged and grounded. Consequently, the particles are attracted to the object, where they adhere and lose their charge. This method of application results in the entire article being evenly coated, thereby yielding increased coverage per gallon of coating composition. Other advantages of this method of application are that it eliminates loss of coating composition from overspray, reduces labor requirements, and reduces air pollution. Wooden workpieces containing more than approximately 10% moisture may be grounded in the same fashion as metal objects and may be sprayed electrostatically.

Since this unique application requires that the coating particles be electrically charged, electrical conductivity is an essential property of the coating material. Moreover, the coating material must have electrical conductivity within a certain range to facilitate proper coating. This range varies with the type of coating material. Most coating compositions do not inherently possess this required degree of electrical conductivity. Therefore, substances which impart electrical conductivity must be added to the coating. Presently, coating compositions contain as much as 30% expensive polar solvent additives such as methylethyl ketone, methanol and nitromethane in order to increase their conductivity to an acceptable level.

The novel electrostatic conductivity additives of the invention comprise oil-soluble sulfonates, water and polar solvent. Although the addition of either polar solvents or mixtures of oil-soluble sulfonates plus water to base coating compositions would alone increase their conductivities, it has been found that additive compositions containing all three of the aforementioned substances remarkably increase conductivities of coating compositions. In addition, it has been determined that the weight ratio of water to oil-soluble sulfonate is critical to the stability of these compositions. Mixtures having water to sulfonate weight ratios of from about 0.3 to about 2.0, that is, 0.3:1 to 2.0:1, do not separate into distinct phases at normal temperatures and are more effective than other mixtures. Thus, compositions having such water to sulfonate ratios are more easily handled and blended with base coating compositions. For this reason a preferred embodiment of the invention is compositions comprising oil-soluble sulfonates, water and polar solvents having water to oil-soluble sulfonate ratios of the above-described range. Particularly preferred are compositions consisting essentially of from about 30 to 70 weight percent oil-soluble sulfonate, from about 20 to 65 weight percent water, and from about 5 to 50 weight percent polar solvent.

2

Generally the sulfonate proportion of the novel additives can consist of any oil-soluble sulfonate. However, sulfonates selected from the group consisting of alkali, alkali earth, and amine salts of oil-soluble sulfonates are preferred. Particularly preferred is sodium mahogany sulfonate.

Any typical organic solvents which have polar characteristics may be used in the additive composition. Examples of these solvents are esters, amides, ketones, alcohols, nitroaromatics, and nitroparaffins. Particularly suitable are polar solvents selected from the group consisting of alkyl ketones, alkyl alcohols, and nitroparaffins. Preferred species of these three classes are alkyl ketones having from 1 to 8 carbon atoms, alkyl alcohols having from 1 to 8 carbon atoms and nitroparaffins having from 1 to 4 carbon atoms. Methanol, methylethyl ketone and nitromethane are particularly preferred because of their excellent polar qualities and commercial availability.

20 Due to their remarkable conductivity enhancing qualities, only small amounts of the new additives are required to adjust the conductivities of coating compositions to levels acceptable for electrostatic application. Consequently, these novel conductivity additives greatly reduce the amount of conventional polar solvent necessary to adjust conductivity. Either all or the bulk of the expensive polar solvents presently used may be replaced by inexpensive hydrocarbon solvents which may be chosen based on their volatility and solvent power rather than 25 their conductivity inducing properties.

The great majority of industrial coating compositions electrostatically applied are baking enamels which have some initial conductivity. It has been found that the conductivity of these enamels may be adjusted to optimum 30 value for electrostatic application by the addition of less than 1% of the new additives. Other industrial coating compositions such as air-drying enamels, which have essentially no initial conductivity, may require the addition of about 3% of the new additive with a few percent 35 conventional polar solvent to bring their conductivity to a satisfactory level. However, the amount of conventional polar solvent necessary to adjust conductivity is always much less than would be required without the addition of the new additives of the invention. Neither 40 the viscosities nor other properties of coating compositions are disturbed by the addition of the new additives. In addition, the new additives present storage advantages (less volume) and eliminate the odor problems involved 45 in using conventional polar solvents.

50 Table I contains various additive compositions and is a tabulation of the additives tested in the following Table II.

Table II illustrates the comparison between the 55 amounts of a commonly used polar solvent, methylethyl ketone, and amounts of various new additive composition required to achieve a Ransburg resistance of 0.2 megohms in coating compositions. Since Ransburg resistance is inversely related to conductivity, the former may 60 be used to determine the acceptability of coating materials for electrostatic application. In fact, Ransburg resistance as determined with a Ransburg resistance meter is the commonly used measure of acceptability for electrostatic application. This meter is essentially an ohmmeter adapted to measure the electrical resistance through a 65 fixed volume of coating composition. On the Ransburg resistance scale one megohm represents 125 megohm-cm. of specific resistivity. The desirable coating-resistance range recommended by Ransburg for electrostatic application is 0.1 to 1.0 megohms. However, the optimum resistance may vary with the individual coating 70 compositions and their end uses.

3  
TABLE I

| Designa-<br>tion | Additive Composition (weight percent)             |                              |       | 5  |
|------------------|---------------------------------------------------|------------------------------|-------|----|
|                  | Sulfonate                                         | Polar solvent                | Water |    |
| A                | Sodium mahogany sulfonate, 50.0.                  | Methylcetyl ketone, 25.0.    | 25.0  |    |
| B                | Calcium mahogany sulfonate, 33.3.                 | Methylethyl ketone, 33.3.    | 33.3  |    |
| C                | do                                                | Methanol, 33.3               | 33.3  |    |
| D                | Ethylene diamine dodecyl benzene sulfonate, 33.3. | Methylethyl ketone, 33.3.    | 33.3  | 10 |
| E                | do                                                | Methanol, 33.3               | 33.3  |    |
| F                | Sodium mahogany sulfonate, 50.0.                  | Methylisobutyl ketone, 25.0. | 25.0  |    |
| G                | do                                                | Methylisamyl ketone, 25.0.   | 25.0  |    |
| H                | do                                                | Diisobutyl ketone, 25.0.     | 25.0  | 15 |
| I                | do                                                | Nitropropane, 25.0           | 25.0  |    |
| J                | do                                                | Amyl alcohol, 25.0           | 25.0  |    |
| K                | do                                                | Methylamyl alcohol, 25.0     | 25.0  |    |

TABLE II

| No. | Base coating composition (weight percent)                                                                        |                                                                         |                                                                                   |       | Drying<br>method | Volume percent of conductivity additive required in various coating compositions to achieve Ransburg resistance of 0.2 megohms |                  |          |
|-----|------------------------------------------------------------------------------------------------------------------|-------------------------------------------------------------------------|-----------------------------------------------------------------------------------|-------|------------------|--------------------------------------------------------------------------------------------------------------------------------|------------------|----------|
|     | Pigment                                                                                                          | Binder                                                                  | Volatile solvent <sup>1</sup>                                                     | Misc. |                  | Methyl-<br>ethyl<br>ketone                                                                                                     | Designa-<br>tion | Additive |
| 1   | Titanium oxide, 26.8                                                                                             | Soya alkyd resin, 50.3; melamine formaldehyde resin, 13.9.              | Isopropyl alcohol, 3.9; xylene, 4.9.                                              | 0.2   | Bake             | 4.4                                                                                                                            | A                | 0.9      |
| 2   | Titanium oxide, 4.0; aluminum stearate, 0.2; lemon yellow oxide, 7.2; chrome green medium, 0.7; lamp black, 0.4. | Dehydrated castor alkyd resin, 46.9; urea formaldehyde resin, 20.2.     | Aromatic hydrocarbons B.R. 360-400° F., 6.9; denatured alcohol, 3.4; xylene, 4.9. | 0.1   | do               | 7.4                                                                                                                            | A                | 0.9      |
| 3   | Titanium oxide, 26.7                                                                                             | Styrenated alkyd resin, 48.6; melamine formaldehyde resin, 17.0.        | Xylene, 3.7; n-butanol, 13.7.                                                     | 0.4   | do               | 1.5                                                                                                                            | A                | 0.15     |
| 4   | Titanium oxide, 24.6                                                                                             | Dehydrated castor alkyd resin, 44.3; melamine formaldehyde resin, 23.7. | Xylene, 3.5; n-butanol, 3.5.                                                      | 0.4   | do               | 3.4                                                                                                                            | A                | 0.6      |
| 5   | Titanium oxide, 31.9; zinc oxide, 2.3.                                                                           | Styrenated alkyd resin, 61.0.                                           | Xylene, 3.2                                                                       | 1.8   | Air-dry          | 17.0                                                                                                                           | A                | (2)      |
| 6   | Titanium oxide, 29.0                                                                                             | Soya alkyd resin, 46.4                                                  | Aromatic hydrocarbons B.R. 280-330° F., 23.2.                                     | 1.4   | do               | 29.0                                                                                                                           | A                | (3)      |
| 7   | (4)                                                                                                              | Long oil alkyd resin, 30.0                                              | Aromatic hydrocarbon B.R. 280-330° F., 70.0                                       | 0.0   | do               | 30.0                                                                                                                           | B                | 4.4      |
| 8   | (4)                                                                                                              | do                                                                      | do                                                                                | 0.0   | do               | 30.0                                                                                                                           | C                | 3.4      |
| 9   | (4)                                                                                                              | do                                                                      | do                                                                                | 0.0   | do               | 30.0                                                                                                                           | D                | 5.9      |
| 10  | (4)                                                                                                              | do                                                                      | do                                                                                | 0.0   | do               | 30.0                                                                                                                           | E                | 5.2      |
| 11  | Titanium oxide, 4.0; aluminum stearate, 0.2; lemon yellow oxide, 7.2; chrome green medium, 0.7; lamp black, 0.4. | Dehydrated castor alkyd resin, 46.9; urea formaldehyde resin, 20.0.     | Aromatic hydrocarbons B.R. 360-400° F., 6.9; denatured alcohol, 3.4; xylene, 4.9. | 0.1   | Bake             | 7.4                                                                                                                            | F                | 1.2      |
| 12  | do                                                                                                               | do                                                                      | do                                                                                | 0.1   | do               | 7.4                                                                                                                            | G                | 1.4      |
| 13  | do                                                                                                               | do                                                                      | do                                                                                | 0.1   | do               | 7.4                                                                                                                            | H                | 1.4      |
| 14  | do                                                                                                               | do                                                                      | do                                                                                | 0.1   | do               | 7.4                                                                                                                            | I                | 1.0      |
| 15  | do                                                                                                               | do                                                                      | do                                                                                | 0.1   | do               | 7.4                                                                                                                            | J                | 1.4      |
| 16  | do                                                                                                               | do                                                                      | do                                                                                | 0.1   | do               | 7.4                                                                                                                            | K                | 1.5      |

<sup>1</sup> B.R. = Boiling range.<sup>2</sup> 4%+2% methanol.<sup>3</sup> 4%+3% methanol.<sup>4</sup> Pigments, which display no effect upon conductivity, were omitted.

Basically, coating compositions consist of pigments, volatile solvents and organic binders. Pigments are finely powdered materials which are practically insoluble in the binder. The type of pigment used depends upon the color, opacity and filling properties desired to be imparted to the coating composition. The volatile solvent is used to reduce the coating composition viscosity to a level at which the composition can be satisfactorily applied. Volatile solvents include a variety of organic liquids whose use varies with their commercial availability and the solubility characteristics of the particular binder being employed in the composition. Examples of some commonly used volatile solvents are mineral spirits, toluene, n-butanol, xylenes, etc. The binder is an organic material, usually a resin or oil, which binds the pigment particles into a coherent film and provides the necessary adhesion of that film to the surface on which it is applied. The end use of the coating composition is primarily dependent upon the nature of the binder con-

stituent. For this reason, coating materials are generally classified according to their binder component. Minor components such as drying agents, antiskinning agents, wetting agents, and the like may be incorporated into the coating compositions depending upon the desired end properties.

Coating compositions susceptible to electrostatic application are those whose viscosity can be adjusted to spraying consistency. These coatings include those based on oleoresinous varnishes, alkyd resins, amino resins, phenolic resins, chlorinated rubber resins, rubber resins, acrylic ester resins, cellulosic resins, vinyl resins and waxes. These coating compositions combined with oil-soluble sulfonates, water and polar solvents constitute novel electrostatic coating compositions. A variety of means can be employed to incorporate these substances into the base composition. Stable mixtures of oil-soluble sulfonates plus water having weight ratios of water to sulfonate of from about 0.3 to 2.0 can be added followed

by the addition of an amount of polar solvent necessary to obtain a desirable conductivity level.

The following examples illustrate the effectiveness of this particular method.

#### Example 1

A coating composition containing 800 g. titanium oxide, 1280 g. medium oil alkyd resin, 1540 g. aromatic hydrocarbons having a boiling range from 280 to 330° F., 65 16 g. calcium naphthenate, 8 g. cobalt naphthenate, 19 g. lead naphthenate and 4 g. antiskinning agent was compounded. To approximately 290 ml. of this composition 1.3 ml. of a 1:1 solution by weight of water to sodium mahogany sulfonate was added. The Ransburg resistance of this mixture was adjusted to 1.1 megohms by the addition of 25.0 ml. methylethyl ketone. When methylethyl ketone alone is added 123 ml. of the ketone is required to adjust the Ransburg resistance to 1.1 megohms.

*Example II*

A base coating composition containing 800 g. titanium oxide, 1280 g. medium oil alkyd resin, 1240 g. aromatic hydrocarbons having a boiling range from 280 to 330° F., 16 g. calcium naphthenate, 8 g. cobalt naphthenate, and 4 g. antiskinning agent was compounded. To approximately 290 ml. of this composition 0.9 ml. of a 1:1 solution by weight of water to sodium mahogany sulfonate was added. The Ransburg resistance of this was adjusted to 1.1 megohms by the addition of 15.0 ml. methanol. Approximately 19 ml. of methanol by itself is required to adjust the resistance of 290 ml. of this coating composition to 1.1 megohms.

*Example III*

To 290 ml. of the base coating composition of Example II, 0.9 ml. of a 1.1 solution by weight of water to sodium mahogany sulfonate was added. The Ransburg resistance of this mixture was adjusted to 1.1 megohms by the addition of 24.0 ml. of nitromethane. Approximately 36 ml. of nitromethane by itself is required to adjust the resistance of 290 ml. of this coating composition to 1.1 megohms.

A preferred method is to directly incorporate conductivity additive compositions comprising all three substances. Such a method was used to obtain most of the data contained in Table II. Either method results in novel coating compositions comprising a major proportion of a base coating composition of sprayable viscosity and a minor proportion of from about 0.1 to 2.0 volume percent oil-soluble sulfonate, from about 0.03 to 2.0 volume percent water and from about 0.03 to 10 volume percent polar solvent. The expressed volume percentages are based upon the total coating composition. The preferred method results preferably in novel coating compositions comprising a major proportion of base coating composition and a minor proportion sufficient to enhance the electrical conductivity of the composition of the conductivity additive consisting essentially of from about 30 to 70 weight percent oil-soluble sulfonate, from about

of evaluating coating performance. One such testing method consists of spraying coating compositions with the Ransburg electrostatic hand spray gun fixed six inches from a grounded metal sheet and evaluating the resulting spray patterns. A satisfactory spray pattern should be a sharply defined "doughnut" having a diameter of from 15 to 20 inches, and a small void spot in the center. There should be a minimum of droplet scattering and fine atomization should be apparent at the outer edge of the pattern. Spray patterns for urea alkyd resin enamels containing the new conductivity additives were of fine quality.

The durability of the coating film is one of its most important properties. Electrostatic spraying is simply an application technique, and any constituent added to improve conductivity should have no effect on the inherent protective qualities of the applied coating. The data in Table III show that the additives of the present invention have no detrimental effect on weatherability, adhesion, or hardness of the coating films formed by the test coatings.

Weatherability of the coating films was determined by exposing them to ultraviolet radiation and moisture at room temperature in an Atlas Weather-Ometer for 144 hours and measuring the change in gloss at 16-hour intervals.

Hardness was measured with the Sward hardness rocker according to the method described in the Paint Testing Manual, 12th Edition, 1962, by H. A. Gardner and G. G. Sward, page 138. The value shown in Table III is the number of swings multiplied by 2. The higher the number, the harder the film.

Adhesion was determined by an adhesive tape method, also described in the Paint Testing Manual, page 165. The method involves scribing a cross in the paint film, applying a piece of tape over the cross, and pulling the tape off. The adhesion is rated on a scale from 1 to 10, depending upon the amount of the paint that is removed with the tape. The highest number indicates the best adhesion.

TABLE III

| Coating composition <sup>5</sup> | Gardner 60° gloss <sup>1</sup> |                               | Adhesion rating <sup>2</sup> |                  | Sward hardness <sup>3</sup> |                  |
|----------------------------------|--------------------------------|-------------------------------|------------------------------|------------------|-----------------------------|------------------|
|                                  | Before weathering              | After weathering <sup>4</sup> | Before weathering            | After weathering | Before weathering           | After weathering |
| 1-Additive A                     | 93<br>93                       | 87<br>91                      | 2<br>2                       | 8<br>8           | 44<br>40                    | 32<br>30         |
| 2-Additive A                     | 89<br>82                       | 85<br>80                      | 9<br>9                       | 9<br>9           | 18<br>22                    | 28<br>24         |
| 3-Additive A                     | 85<br>77                       | 82<br>77                      | 1<br>1                       | 9<br>9           | 34<br>32                    | 24<br>26         |
| 4-Additive A                     | 93<br>93                       | 93<br>93                      | 2<br>1                       | 4<br>4           | 36<br>44                    | 32<br>32         |
| 5-Additive A                     | 91<br>84                       | 87<br>80                      | 2<br>2                       | 7<br>7           | 44<br>44                    | 22<br>20         |

<sup>1</sup> Highest number is highest gloss.

<sup>2</sup> 1 is poor; 10 is good.

<sup>3</sup> Highest number is hardest film.

<sup>4</sup> 144 hours in Weather-Ometer.

<sup>5</sup> Coating compositions are those corresponding to Nos. 1-5 in Table II and containing enough of the designated additive to achieve a Ransburg resistance of 0.2 megohm.

20 to 65 weight percent water and from about 5 to 50 weight percent polar solvent selected from the group consisting of alkyl ketones, alkyl alcohols and nitro-paraffins. If the latter method is employed, a preferred range for said minor proportion is from about 0.1 to 4.0 volume percent of the total coating volume.

The ultimate effectiveness and value of both the additives and the novel coating compositions containing the additives is gauged by the protective and decorative qualities of the new coating compositions. Functional testing of coatings is perhaps the most conclusive method

65 The foregoing detailed description has been given for clearness of understanding only and no unnecessary limitations are to be understood therefrom. The invention is not limited to the exact details shown and described for obvious modifications will occur to those skilled in the art.

70 We claim:

1. A novel electrostatic coating conductivity additive composition consisting essentially of from about 30 to 70 weight percent sodium salt of mahogany petroleum sulfonic acid, from about 20 to 65 weight percent water and from about 5 to 50 weight percent of polar solvent selected

from the group consisting of alkyl ketones having from 1 to 8 carbon atoms in the alkyl groups, alkyl alcohols having from 1 to 8 carbon atoms and nitroparaffins having from 1 to 4 carbon atoms, the weight ratio of said water to said sulfonic acid sodium salt being from about 0.3:1 to about 2.0:1.

2. The additive composition of claim 1 in which the polar solvent is methylethylketone.

3. The additive composition of claim 1 in which the polar solvent is nitromethane.

4. The additive composition of claim 1 in which the polar solvent is methanol.

5. A novel electrostatic coating composition comprising a base coating composition of sprayable viscosity and from about 0.1 to 4.0 volume percent of the additive composition of claim 1.

5

10

6. The coating composition of claim 5 in which the polar solvent is methylethylketone.

**References Cited by the Examiner**

**UNITED STATES PATENTS**

|           |         |          |       |          |
|-----------|---------|----------|-------|----------|
| 2,419,048 | 4/1947  | Althouse | ----- | 260—29.2 |
| 2,723,921 | 11/1955 | Starkey  | ----- | 117—93.4 |
| 3,112,218 | 11/1963 | Spiller  | ----- | 117—93.4 |

**OTHER REFERENCES**

"Concise Chemical and Technical Dictionary," Bennett, Chemical Publishing Co., Inc., Brooklyn, N.Y., 1947, QD5B4, p. 577.

15 SAMUEL H. BLECH, *Primary Examiner*.